

## UNITED STATES PATENT OFFICE

2,642,350

## METHOD OF RECLAIMING SINGLE BASE SMOKELESS POWDER

Dwight A. Alderson, East Alton, Ralph Vincent Wakefield, Roxana, and Emerald P. Reichardt, Wood River, Ill., assignors to Olin Industries, Inc., East Alton, Ill., a corporation of Delaware

No Drawing. Application August 9, 1950,  
Serial No. 178,558

4 Claims. (Cl. 52—20)

1

This invention relates to a process for reworking smokeless powder and more particularly to a process for reclaiming the nitrocellulose content from single base smokeless powders having a substantial content of a modifier.

Government surplus cannon powders known as non-hydroscopic (NH), and flashless non-hydroscopic (FNH) smokeless powders and powders known to the trade as IMR type, such as cal .30, cal. .50, and 20 mm. have as their base nitrocellulose of about 13.2% nitrogen content. Nitrocellulose of such nitrogen content is well suited for use as a raw material for making smokeless powders for sporting cartridges. However, such types of smokeless powder are not readily reworked into sporting cartridge powder due to their high content of modifiers, e. g. NH powder has about 8% dinitrotoluene and 4% dibutylphthalate. When such type powders are used as the raw material in a process such as that set forth in U. S. 2,027,114, issued January 7, 1936, to Fredrich Olsen et al., the resulting smokeless powder is dirty burning, that is to say, a residue of incompletely burned powder grains is left in the barrel of the gun. This objectionable feature is believed to arise from the fact that the presence of deterrent materials within the resulting sporting powder grain inhibits the burning of such grains to the extent that a number of the grains, or parts thereof, of a charge are not fully burned. In addition to this dirty burning effect the deterrent materials within the powder grain reduces the propellant power of the powder.

It is therefore an object of this invention to provide a novel process for reworking such single base powders as are represented by the NH, FNH and IMR powders to provide a suitable base material for use in the manufacture of powder for sporting ammunition, military ammunition, and the like. Another object is to provide a safe economical process for producing raw material for clean burning smokeless powders.

The foregoing objects and advantages as well as others which may become apparent from the detail description hereinafter are accomplished in accordance with this invention by treating the smokeless powder to be reclaimed in a mixture of benzol and water. It has been discovered that by agitation and heating of the particulate powder while immersed in a mixture of benzol and water, a portion of the modifying material is removed and the residue is so uniformly distributed through the powder that the aforementioned objectionable features are eliminated. By

2

particulate powder as used herein is meant single base cannon powders as exemplified by the 20 mm., FNH and NH types ground to a particle size of not more than about 10% held in a standard U. S. 0.070 inch screen and ground or unground .30 cal. and .50 cal. IMR type powder having a relatively high content of dinitrotoluene and dibutylphthalate, or similar modifiers. The treated particulate powder is then a source of clean, high nitrogen cellulose suitable for use as a raw material for the manufacture of smokeless powders by processes such as that set forth in the aforementioned U. S. Patent 2,027,114.

In carrying out the process the cannon powder is preferably ground in a water slurry to a particle size substantially within the range of about 0.07 inch to 0.004 inch in diameter. The particulate powder is then agitated in a mixture of from about 4 to 8 parts benzol and a minimum of 2 parts water per part of powder at a temperature in the range from 30° C. to the boiling point of benzol but preferably not above about 65° C. for a period of at least four hours' duration. At the end of the treatment the powder is separated from the aqueous benzol emulsion by any suitable means such as decantation, centrifuging or vacuum filtration. Any residual benzol adhering to the separated powder, which in some instances may be as high as 0.7 part benzol per part powder, may readily be removed by again adding a minimum of about 2 parts water per part of powder and heating the slurry to a temperature around the boiling point of water, for example 99° C., while permitting the benzene to escape from the system. The water wet powder may then be dried, if desired, or may be utilized in the water wet condition as the nitrocellulose for the process set forth in the aforementioned U. S. Patent 2,027,114. It is not essential that the treatment with aqueous benzol completely remove the modifier content which is ordinarily composed of dinitrotoluene and dibutylphthalate, but the duration of the treatment should be such that the residue of such material is less than about 2% by weight of the powder. It has been found that when the treatment is of such duration the powder is properly conditioned for conversion into smokeless powder of satisfactory burning characteristics. It is preferable to carry out the treatment in two or more steps. For example, the first step may consist of a treatment of four hours' duration after which the powder is separated from the benzol emulsion and the powder is then again treated in a fresh mixture of benzol and water for another four hour pe-

riod after which the process is completed as set forth above. In the treatment, the solvent power of the benzol constituent is most effective in removing the undesirable modifiers, although the water effects some improvement in this removal. The water has also a number of other beneficial effects such as one of dilution so that each particle gets a more uniform treatment. The water also tends to reduce the amount of benzol adherent to the powder grains after the treatment. However, an important function of the water is to increase the safety of the operation. For example, if during the treatment, for one cause or another, the benzol should take fire, the powder being treated is not likely to be 15 fired and the hazard is greatly minimized. In the absence of the water, a benzol flash would be followed by a firing of the powder being treated. Furthermore, the last traces of benzol are more difficultly removable in the absence of the water. 20

In order to further clarify the invention there follows a detailed description of a preferred embodiment thereof.

*Example I*

Cannon powder of the NH type is ground water wet, for instance in a Dixie hammer mill, to a particle size such that a minimum of about 90% of the ground powder passes through a 0.07 inch screen and a maximum of about 3% passes through a 0.0046 inch screen. One part of such ground powder is then charged with 2.2 parts of water and 4 parts of benzol by weight into an extraction kettle and the mixture is agitated at a speed that will insure a uniform dispersion of the powder, water and benzol. The mixture is heated as rapidly as possible during the agitation to a temperature of 65° C. and maintained with agitation at this temperature for about four hours. At the end of the four hour period, the water-benzol emulsion is removed from the powder by vacuum filtration. A fresh charge of benzol and water in the same ratios utilized above are then added to the powder in the kettle and the mixture is again heated with agitation as rapidly as possible to 65° C. and the temperature maintained there for about four hours. The benzol-water emulsion is then removed from the powder as above by vacuum filtration. In order to remove the last traces of benzol from the filtered powder, about 2.5 to about 3.0 parts by weight of water are added to the powder. The mixture is then agitated as above and heated as rapidly as possible to 99° C. and this temperature is maintained for about 30 to 45 minutes to remove the benzene from the system. The mixture is then cooled to a temperature less than about 65° C. and the water is removed from the powder by decantation or vacuum filtration. The powder may then be dried, if it is so desired, or it may be utilized in the water wet state as the raw material for a process such as that set forth in U. S. Patent 2,027,114.

As an illustration of the effectiveness of such treatment, the powder before treatment had an ether extractable content of about 13.5%, whereas as after the treatment the ether extractable content was only about 1.4%. The ether extractable content of the untreated powder included about 8.6% dinitrotoluene and about 3.8% dibutyl-phthalate.

*Example II*

In another embodiment the powder was treated as described in the foregoing example with the exception that 8 parts of benzol were used for

each part of powder instead of four parts, and in this instance the treated powder had a residual ether extractable content of about 1.6%.

*Example III*

In still another embodiment the powder was treated as set forth in Example I except that the powder was treated four times with the benzol-water emulsion instead of two and at a temperature of 60° C. instead of 65° C. After treatment the residual ether extractable content of powder was 1.27%.

*Example IV*

In still another embodiment the powder was treated as set forth in Example I except that the benzol to powder ratio was about 3 to 1, instead of 4 to 1, and only a single treatment was given with the emulsion at a temperature of 60° C. The treated powder then had an ether extractable content of about 1.7%.

As illustrated in the foregoing embodiments, this invention accomplishes its purpose of substantially reducing the modifier content of the treated powder and the treated powder is then in a suitable condition for reprocessing. If amounts of benzol greater than about 8 parts to 1 part of powder are utilized, no appreciable benefit is effected in the treatment and the process becomes uneconomical and more hazardous. Amounts of benzol substantially less than 4 parts to 1 part of powder are not satisfactory from the standpoint of removing the undesirable modifiers and reconditioning the powder. If less than about 4 parts benzol are utilized, the number of extractions must be increased and even then one cannot be certain of obtaining a useful product. However, while certain specific details are set forth herein, it should be understood that considerable modification can be made without departing from the spirit and scope of the invention.

Having thus described the invention, what is claimed and desired to secure by Letters Patent is:

1. The method of reclaiming single base smokeless powder containing benzol-soluble modifiers which consists in dispersing the powder in particulate form in a mixture composed essentially of benzol and water, agitating the mixture at an elevated temperature until a substantial portion of the modifier content is dissolved, removing the benzol-water mixture from the powder, adding water to the powder and heating until the residual benzol is removed from the powder and thereafter cooling the mixture.

2. The method of reclaiming single base smokeless powder containing benzol-soluble modifiers which consists in dispersing the powder in particulate form in a mixture composed essentially of about four to eight parts benzol and a minimum of about two parts water per part of powder at a temperature in the range from about 30° C. to the boiling point of the benzol, agitating the mixture for at least about four hours, separating the powder from the benzol-water mixture, adding water to the powder and heating with agitation of the mixture to a temperature near the boiling point of water until the residual benzol is removed from the powder, and thereafter cooling the mixture.

3. The method of reclaiming single base smokeless powder containing benzol-soluble modifiers which consists in dispersing the powder in particulate form in a mixture composed essentially

of about four parts benzol and about two parts water per part of powder at a temperature of about 65° C. for a period of about four hours and then separating the powder from the benzol-water mixture, repeating said treatment until the modifier content of said powder has been reduced to less than about 2% by weight of the powder, dispersing said powder in water and heating the mixture to a temperature near the boiling point of the water until the benzol is removed from the powder and thereafter cooling the mixture. 10

4. The method of reclaiming single base smokeless powder containing benzol-soluble modifiers by dispersing one part of powder in particulate form in a mixture composed essentially of at least four parts of benzol and at least two parts of water at a temperature below the boiling point 15

of the benzol with agitation for at least four hours, removing the benzol-water mixture from the powder, adding water to the powder and heating until the residual benzol is substantially removed from the powder.

DWIGHT A. ALDERSON.  
RALPH VINCENT WAKEFIELD.  
EMERALD P. REICHARDT.

## References Cited in the file of this patent

## UNITED STATES PATENTS

| Number    | Name         | Date          |
|-----------|--------------|---------------|
| 1,439,656 | Woodbridge   | Dec. 19, 1922 |
| 1,666,049 | Tozier       | Apr. 10, 1928 |
| 2,123,517 | Woodbridge   | July 12, 1938 |
| 2,151,494 | Ball         | Mar. 21, 1939 |
| 2,175,212 | Olsen et al. | Oct. 10, 1939 |